

P. ZADIG.  
Cobble Stone-Pavements.

No. 154,999.

Patented Sept. 15, 1874.

Fig 1.



Fig 2.



Fig 3.



Witnesses.  
H. L. Moutteverde.  
Raymond Gibbons.

Inventor  
Philip Zadig  
By his Atty  
C. W. M. Smith.

# UNITED STATES PATENT OFFICE.

PHILIP ZADIG, OF SAN FRANCISCO, CALIFORNIA.

## IMPROVEMENT IN COBBLE-STONE PAVEMENTS.

Specification forming part of Letters Patent No. 154,999, dated September 15, 1874; application filed August 22, 1874.

*To all whom it may concern:*

Be it known that I, PHILIP ZADIG, of San Francisco, county of San Francisco and State of California, have invented an Improvement in Concrete or Stone Blocks for Pavements, and molds or flasks for forming the same; and I do hereby declare that the following is a full, clear, and exact description of the same, reference being had to the accompanying drawings and to the letters marked thereon.

This invention relates to an improved construction of block for paving streets; also to an improved flask in which the blocks are molded. It consists mainly in providing a concrete block with elevation and depression or corrugations, to afford a better foot-hold for animals.

The flask in which the block is formed differs essentially from that described in my former specification, for which Letters Patent were granted to me July 25, 1874, from the fact that I divide the flask vertically to its base, which admits of the two parts forming the sides and ends to be removed, and leaves the block, when formed and set, upon the base-board or bottom of the mold. The bottom of the mold is provided with semi-oval depressions, so that when the block is removed, oval ridges will remain upon its face, all of which will hereinafter more fully appear.

Referring to the accompanying drawings forming a part of this specification, Figure 1 is a side sectional elevation of my improved flask; Fig. 2, a plan; Fig. 3, a side elevation, in section, of the block.

In my present construction of flasks, A represents a removable base, provided with a raised center and grooved center, B, around which center the sides of the flask fit closely. Two of these sides C, which form the compartment, are entire, while the adjoining two are divided vertically to the base-plate, as shown, and are made with tongues and grooves D, so that the sides of the flask can be easily removed, and leave the composition or concrete of which the paving-block is formed upon the raised and corrugated portion B of the base-plate. These divisions are kept in place by hooks and eyes or clamps E, attached to the sides and base-plate of the flask.

The flasks I construct of wood, lined with zinc plates, the four sides being about six inches high, or of a height sufficient to hold the cobbles, when in position, a little above the point of the largest swell or circumference.

The grooved bottom B should be made of hard wood, and well polished, and sprinkled with lime sweepings, and the sides of the box coated with a solution of lime before using, to prevent adhesion of the material employed.

The following is a description of the block: I take asphaltum, mixed in the general way for giving it the necessary softness, and add to it about fifteen per cent. of pulverized lime-rock, serpentine rock, or chalk-rock, in order to impart the requisite hardness to resist the rays of the sun; then mix with this mass a good proportion of coarse gravel and pebbles, and boil the whole a sufficient length of time, in order that all the particles of the same be well coated with the mixture of the asphaltic compound. I now put the molds in position, and begin with pouring upon the bottom a quarter of an inch of dry fine gravel. After that I fill the bottom with cobble-stones, pressing them down between the fine gravel upon the bottom of the mold.

The cobbles may be of different sizes and shapes, but in a mold six inches deep they ought not to be broader than three and a half nor higher than five and a half inches. I begin by pouring the most liquefied part of the asphaltum upon and between the stones, making sure that it penetrates all the minutest parts of the fine gravel, and continue the filling with coarser parts of the mass, so that the pebbles or coarser portion is laid upon and between the upper half of the cobbles, and avoid as much as possible to build upon the last half inch of the mold or block anything but fine gravel, so that there be no projections on the top, because the top of the mold will form the base or foundation of the block when laid down.

Care should be taken that the platform of the floor upon which the mold is standing when filled be placed in a horizontal and level position. After three hours' cooling the mold or flask can be taken off.

At any time before filling again the sides and bottom of the mold should receive a new coating of lime in solution.

After the mold has been taken off, the block is ready to be laid, and is to be turned bottom up, so that the groove will be upon its upper face, as shown in Fig. 3.

The blocks, as I make them, ten by twenty-two inches by six inches deep, are laid with spaces of two inches, between which spaces, after the street is laid out, are filled with pebbles of about one inch and a half in dimension, and hot asphaltum mixed with tar poured upon it. The above space is preferable, in order to give the liquid a better chance to penetrate to the bottom and fill the gap. By this construction a block is made of great durability and strength, possessing the advantage also of being prepared at the factory in advance for future use.

Having thus described my invention, what

I claim as new, and desire to secure by Letters Patent, is—

1. A block for pavements, composed of cobble-stones with a grooved or corrugated surface, when the same is constructed, and built up in the manner and of the materials as herein set forth and specified.

2. A flask in which to form or mold concrete blocks, whose sides C are divided and removable, substantially as described and shown.

3. In a flask for molding concrete blocks, a removable base, A, provided with a corrugated or grooved surface, B, substantially as and for the purpose described.

In witness whereof I have hereunto set my hand and seal.

PHILIP ZADIG. [L. s.]

Witnesses:

C. W. M. SMITH,  
E. V. SUTTER.